

July 28, 1925.

1,547,363

A. A. CATLIN ET AL

METHOD FOR TREATING CONDUCTORS

Filed Oct. 31, 1919



Fig. 1



Fig. 2



Fig. 3



Inventors

Arthur A. Catlin

Henry R. Massingham

by *J. G. Roberts* Atty

## UNITED STATES PATENT OFFICE.

ARTHUR A. CATLIN, OF EAST ORANGE, NEW JERSEY, AND HENRY R. MASSINGHAM, OF CICERO, ILLINOIS, ASSIGNORS TO WESTERN ELECTRIC COMPANY, INCORPORATED, OF NEW YORK, N. Y., A CORPORATION OF NEW YORK.

## METHOD FOR TREATING CONDUCTORS.

Application filed October 31, 1919. Serial No. 334,852.

*To all whom it may concern:*

Be it known that we, ARTHUR A. CATLIN and HENRY R. MASSINGHAM, citizens of the United States, residing at East Orange, in the county of Essex and State of New Jersey, and at Cicero, in the county of Cook and State of Illinois, respectively, have invented certain new and useful Improvements in Methods for Treating Conductors, of which the following is a full, clear, concise, and exact description.

This invention relates to flexible conductors and more particularly to a method for treating flexible insulated conductors to insure greater life in service. In connection with flexible conductors, such as used, for example, in telephone switchboards for interconnecting the various lines, it is necessary that the outer braiding be capable of withstanding severe service in order that a satisfactory life may be obtained from the cords. Moreover, the ends of these cords to which the connecting plugs are attached are subjected to particularly severe treatment due to the sharp bending of the cord at this point and also due to the perspiration from the hands of the operator. It has been proposed to treat such cords by dipping them in various types of wax in order to prevent moisture from entering the conductors and thereby decreasing the insulating resistance. Cords so treated are not only sticky and stiff but the saturation of the braiding with the impregnating compound lowers the tensile strength of the threads of the braiding, thereby decreasing rather than increasing the life of the cord.

It is therefore the object of the present invention to provide a method for treating flexible conductors, whereby the outer braiding of the conductor is impregnated an amount sufficient to insure increased life of the covering without making the conductor stiff or sticky.

A further object is to impregnate the outer covering an amount sufficient to provide a lubrication for the various threads as they rub against each other without saturating these threads to such an extent as to impair their tensile strength.

To accomplish these objects and in accordance with a feature of this invention, there is provided a method of impregnating flexible conductors in which the impregnat-

ing compound only penetrates the outer portion of the textile covering of the conductor, and in which the time of impregnation and the temperature of the compound are such as to preclude the possibility of the threads being saturated to such a point as to impair their tensile strength.

This and other features of the invention may be more clearly understood by referring to the attached drawings, in which Fig. 1 discloses a switchboard cord of a type which may be preferably treated in accordance with the method embodying this invention and having a portion of the braiding cut away to more clearly show its construction; Fig. 2 discloses apparatus satisfactory for performing the invention; and Fig. 3 is a view of the die forming a portion of the apparatus disclosed in Fig. 2.

The type of cord illustrated in the drawing comprises a core consisting of a plurality of insulated conductors 5-5 twisted together and provided with fillers 6-6 laid as shown to insure a more even core. These conductors are prevented from untwisting by means of a wrapping 7 of tape or thread wound about the core in the opposite direction to that in which the conductors are twisted. The conductors terminate at one end in a switchboard plug 8 and the core at this end is provided with a double covering consisting of an outer braiding 9 and an inner braiding 10.

The apparatus disclosed in Fig. 2 comprises a metal tank 11 provided with heating means, such for example as a gas burner 12. Securely fastened to the tank 11 is a hinged die 13, the jaws of which are normally held open by means of the spring 14. However, a foot pedal 15 is provided as shown to draw the jaws together against the tension of spring 14. The tank 11 contains the insulating compound with which it is desired to impregnate the plug end of the cord, this compound consisting preferably of equal parts of beeswax and paraffine. By means of the gas flame 12, the temperature of this insulating compound is maintained between 180° F. and 200° F. In performing the method embodying this invention, the plug end of a cord such as is disclosed in Fig. 1 is immersed in the insulating compound for a period of from 2 to 4 seconds and is then immediately placed

2  
between the jaws of die 13, foot pedal 15 is pressed downward to draw the jaws together and the cord drawn through the die to remove the excess wax from the outer surface. The die 13 being mounted directly on the metal tank 11 is heated to a temperature approaching that of the insulating compound, but, if desired, a conducting member can be provided extending from the die directly into the insulating compound to insure maintaining this die at a temperature which will permit it to efficiently remove the excess compound.

By following the process outlined, the insulating compound impregnates the outer braiding 9 but does not penetrate into the core of the cord. The threads of braiding 9, however, are not saturated with the insulating compound to such an extent as to impair their tensile strength but the outer surface of these individual threads is impregnated an amount sufficient to provide lubrication for the fibers as they are rubbed one over the other upon bending of the cord and also to afford protection against moisture or perspiration entering the cord to affect the insulation resistance of the conductors. By immediately removing all excess wax from the cord following its immersion, the cord is prevented from becoming sticky and thus disagreeable to handle. If the insulating compound is allowed to penetrate into the core, the cord becomes too stiff to be handled satisfactorily, a difficulty which is overcome by following the method of treating described.

What is claimed is:

1. The process of treating a flexible conductor composed of a conducting core to which have been applied an inner and an outer layer of fibrous material, which con-

sists in immersing the conductor in insulating compound, the temperature of the compound and the time of immersion being such that the fibrous material of the outer layer will receive a coating of the insulating compound but will not be saturated to such a degree as to impair its tensile strength, and then immediately removing the excess compound from the outer surface of the outer layer of fibrous material.

2. The process of treating a flexible conductor which consists in applying thereto an inner and an outer layer of fibrous insulating material, immersing for a period of from two to four seconds in an insulating compound consisting of equal parts of beeswax and paraffine, the temperature of which is not less than 180° F. nor more than 200° F., and then immediately passing through a die to remove excess compound from the outer layer of fibrous material.

3. The process of treating a flexible conductor composed of a conducting core to which have been applied an outer and an inner layer of fibrous material, which consists in immersing the conductor in an insulating compound, the temperature of which is maintained between 180° and 200° F., for a period of time such that the insulating compound will impregnate the outer layer without saturating the fibrous material to such a degree as to impair its tensile strength and without penetrating the core, and then passing the conductor through a heated die to remove excess compound from the outer layer of fibrous material.

In witness whereof, we have hereunto subscribed our names.

ARTHUR A. CATLIN.  
HENRY R. MASSINGHAM.